

# UNITED STATES PATENT OFFICE.

AUGUSTE J. ROSSI, OF NIAGARA FALLS, NEW YORK, ASSIGNOR TO THE TITANIUM ALLOY MANUFACTURING COMPANY, OF NEW YORK, N. Y., A CORPORATION OF MAINE.

## ARTICLE COMPOSED OF TITANIUM AND NICKEL ALLOYED TOGETHER AND METHOD OF PRODUCING THE SAME.

1,003,806.

Specification of Letters Patent.

Patented Sept. 19, 1911.

No Drawing.

Application filed January 6, 1911. Serial No. 601,165.

To all whom it may concern:

Be it known that I, AUGUSTE J. Rossi, a citizen of the United States, and a resident of Niagara Falls, in the county of Niagara and State of New York, have invented a certain new and useful Article Composed of Titanium and Nickel Alloyed Together and Method of Producing the Same, of which the following is a specification.

10 It has heretofore been regarded as impossible to produce the binary alloy of titanium with nickel, and the object of my invention is to produce such alloy and to provide methods for its production so simple, economical 15 and reliable as to justify manufacture thereof on industrial scales. I attain these objects as hereinafter described.

It has been asserted heretofore that because of the much higher melting-point of 20 titanium as compared with that of nickel it was impossible to produce a binary alloy of said metals since titanium added to molten nickel would chill and segregate. I have discovered however that the binary alloy of 25 titanium and nickel is producible provided the titanium is brought in nascent state into the presence of the nickel previously reduced to molten state so as to constitute a bath for the reception of the titanium on its re- 30 duction from an oxid thereof.

Alloys of ferric metals, *i. e.* iron and steel with nickel have by now, as well known, attained a position of recognized high utility in the arts as for instance under the designation of "nickel steels." Such alloys are produced by adding to a ferric metal any desired percentage of nickel and melting the two together.

The ferric metal and also the nickel contain 40 impurities, being undesired elements and compounds including slags, etc., which it is desirable should if possible be eliminated. Titanium in quantity proportioned to satisfy the chemical affinities of such undesired elements and compounds is as I have 45 heretofore discovered efficient to insure their removal when added to the ferric bath containing them as an alloy of titanium with ferric metal. I have now discovered that the 50 efficiency of titanium in the particular mentioned is not impaired by its association with nickel as in alloy therewith, and therefore my said novel alloy is of important utility in

that by its addition to baths of molten ferric metal, not only is nickel alloyed with the latter but also both metals and their resulting alloy simultaneously purified by the titanium. Moreover my novel alloy is also particularly useful to so purify molten nickel intended for use by itself alone for other applications in the arts.

My novel alloy of titanium with nickel I produce as follows:—I charge into a graphite crucible or other container properly adapted, nickel, titanic acid, and preferably 65 an oxid of nickel, also such an amount of aluminium (preferably in shots or the like so as to melt more rapidly) as is chemically sufficient to decompose the oxid of titanium and also the oxid of nickel, and reduce their 70 respective titanium and nickel contents to their metallic states. This mixture is then heated, as preferably in any of the well known forms of so called electric furnaces, or otherwise, to a temperature sufficiently 75 high to insure the melting of the metallic element of the charge and the taking place of the required reactions as hereinafter noted. The molten product on being withdrawn and cooled will be found to be an 80 alloy of titanium with nickel, the percentage of the former being proportional to the amounts of titanic acid and aluminium charged, the reactions being as per the following formula, assuming that the oxid of 85 nickel designated as NiO is employed.



While in this instance the presence of 90 an oxid of nickel is not absolutely essential it nevertheless promotes considerably the reactions desired in the charge and accelerates its fusion into a homogeneous metallic alloy, the heat of the formation of 95 such oxid being so much less than that of the oxid of titanium as to leave available a considerable excess of heat due exothermally to the combination of its oxygen with part of the aluminium of the bath. 100 In this manner an alloy of nickel with titanium containing any desired percentage of titanium may be produced. Moreover such use of an oxid of nickel, or even its substitution entirely for the metal in said 105 process, is sometimes economically desir-

able, the cost of such oxid being usually less than that of the metal, and such entire substitution being possible in the production of my said alloy by my said process. I have also discovered that my said alloy of nickel with titanium may, in some instances, be advantageously produced by substituting carbon for aluminium as the reducing agent, in which case it is essential in industrial practice to employ the higher temperatures derivable for instance from some of the now well known forms of so-called electric furnaces, such for example as illustrated and described in Letters Patent No. 802,941 granted to me October 4, 1905. In this case oxid of nickel, oxid of titanium, and carbon are mixed together as for instance as per the formula



Said mixture, together with some nickel, is charged in said furnace and the current turned on. This will result in production 25 of a bath of molten nickel, and, the current being continued, the titanium oxid will be reduced to titanium, which mingles, or absorbs, in said bath of nickel to constitute the alloy. The addition of nickel in metallic state, though not absolutely necessary, facilitates the reduction of the titanium oxid by the carbon. The proportions

of the ingredients used in the charge will be varied according to the percentage of the respective metals desired in the alloy 35 according to the formulas above given and as experience and test in each case will readily demonstrate to those skilled in the metallurgical art.

What I claim as new and desire to secure 40 by Letters Patent is the following, viz:—

1. As a new article an alloy of titanium with nickel.

2. The process of producing an alloy of titanium with nickel which comprises incorporating titanic acid into a bath of molten nickel in presence of a reducing agent, subjecting the bath to a temperature sufficient to insure reduction of said titanic acid by said agent, and withdrawing and 50 cooling the resulting metallic product.

3. The method of producing an alloy of nickel with titanium which comprises incorporating titanic acid into a bath comprising molten nickel and molten aluminium, subjecting the bath to a temperature sufficient to insure reduction of said titanic acid by said aluminium and withdrawing and 55 cooling the resulting metallic product.

AUGUSTE J. ROSSI.

Witnesses:

WALTER D. EDMONDS,  
GEORGE G. MEASURES.